

July 7, 1959

R. T. LOWERRE

2,893,640

RAIL BOND AND METHOD OF INSTALLING THE SAME

Filed March 4, 1954

2 Sheets-Sheet 1

FIG. 1.



FIG. 2.



FIG. 3.



FIG. 4.



FIG. 5.



INVENTOR:  
RALPH T. LOWERRE,

BY: *Donald G. Dalton*  
his Attorney.

July 7, 1959

R. T. LOWERRE

2,893,640

RAIL BOND AND METHOD OF INSTALLING THE SAME

Filed March 4, 1954

2 Sheets-Sheet 2

FIG. 6.



FIG. 7.



INVENTOR:  
RALPH T. LOWERRE,

BY: *Donald G. Dalton*  
his Attorney.

1

2,893,640

RAIL BOND AND METHOD OF INSTALLING  
THE SAME

Ralph T. Lowerre, Bedford, Ohio, assignor to United States Steel Corporation, a corporation of New Jersey

Application March 4, 1954, Serial No. 414,100

4 Claims. (Cl. 238—14.13)

This invention relates to a rail bond and to a method of installing the same and particularly to a rail bond not mechanically attached to the rail. Mechanically attached rail bonds have the disadvantage of being difficult and expensive to apply to the rail. For that reason it has been proposed to weld rail bonds to the rail. While such bonds have been utilized to some extent they also have certain disadvantages which have prevented them from supplanting mechanically applied rail bonds. If the rail is not preheated before welding or heat treated after welding, the heat of the welding operation will cause the structure of the steel in the rail to change to martensite, this being detrimental to rail life. If the rail is preheated prior to installation of the bond, the cost is increased so that there is no advantage over mechanically applied bonds. If the rail is heat treated after welding, the installed bond is damaged and its life seriously impaired.

It is therefore an object of my invention to provide a rail bond which can be readily and inexpensively applied to a rail without prior heating, without postheating after welding, and without drilling the rail as necessary for a mechanically applied bond.

Another object is to provide a method of making and attaching such a rail bond to a rail.

These and other objects will be more apparent after referring to the following specification and attached drawings, in which:

Figure 1 is a top plan view of a bond applied to a rail;

Figure 2 is a view showing the bond in one stage of its manufacture;

Figure 3 is a view of a terminal of the bond prior to its installation;

Figure 4 is a view taken on the line IV—IV of Figure 3;

Figure 5 is a plan view of the equipment used in installing the bond;

Figure 6 is a sectional view taken on the line VI—VI of Figure 5; and

Figure 7 is an end view of the mold of Figure 6 looking from the left hand end thereof.

Referring more particularly to the drawings, the reference numeral 2 indicates a flexible conductor which is preferably a stranded wire structure made of copper or bronze. A copper sleeve 4 is fastened to each end of the conductor 2 and a thin metal buffer plate 6 is fastened to the sleeve 4. Plate 6 has a generally elliptical portion 8 and a sleeve portion 10 which is wrapped around the sleeve 4 and mechanically locked in place. A sheet 12 of material having a relatively low melting point with respect to plate 6, such as solder is attached to the portion 8 by bending its longitudinal edges 14 therearound as shown in Figure 4. Instead of applying the layer of solder mechanically it may be applied as a coating. The plate 6 need not be the exact shape shown, it being understood that it is only necessary to have a portion similar to portion 8 which can be fastened to the sleeve 4 in

2

any suitable manner. For example, instead of the mechanical connection shown the parts may be brazed. The sleeves 4 can also be omitted but are desirable in order to keep the strands of the member 2 from spreading.

5 In assembling the rail bond on the rails R, a mold or a pair of molds 16 are provided. Each mold includes a crucible 18, a sprue 20, and a cavity 22. The cavity 22 is open on the side toward the rail R and has a notch 24 at one end for receiving the sleeve 4 or 10. A counter-sunk portion 26 is provided around the mold cavity adjacent the rail. As shown in Figure 5, two molds 16 are provided so that the bond can be attached to adjacent rail ends at the same time. The molds 16 are attached to a U-shaped member 28 by means of brackets 30, screws 32 and bolts 34. A rod 36 extends from the base of the U-shaped member 28 away from the molds 16. A jaw 38 having a downwardly extending portion 40 is slidably mounted on the rod 36. A nut 42 is mounted on the threaded end of the rod 36. 10 A spring 44 is arranged on the rod 36 between the jaw 38 and a member 46 which bears against the nut 42. In fastening the rail bond to the rail ends the molds 16 are attached to the rail heads adjacent the ends of the rail in the desired position as shown in Figure 5, the body of the molds and the jaw portion 40 gripping the rail head therebetween. The spring 44 serves to urge the jaw 38 toward the molds 16. The force exerted by the spring 44 may be varied by loosening or tightening the nut 42. This adjustment also serves to compensate 15 for different widths of rail heads. It will be understood that the exact construction of the molds 16 and the means for fastening the molds to the rail may vary. Suitable molds and clamping devices are shown in the patents to Cadwell Nos. 2,251,820, dated August 5, 20 1941, 2,262,755, dated November 18, 1941, and 2,276,823, dated March 17, 1942. One of the plates 6 is inserted in the cavity 22 of each of the molds, the plate 6 resting in the counterbored portion 26 with the sleeve 4 or 10 in the opening 24. In this position the solder 25 12 will be in contact with the rail. An exothermic welding mixture 48 is placed in the crucibles 18 with the sprues 20 being closed by means of a destructible seal 50. Ignition of the mixture 48 produces molten welding metal which destroys the seals 50 and discharges into the mold cavity 22 which is shaped to give the desired contour to the terminal fitting. This molten metal forms terminal fitting 52 which is integral with the buffer plate 6 and the end of the conductor 2. The heat of the molten metal in the cavity causes the solder to melt and 30 fuse the plate 6 to the rail R. The buffer plate 6 is thin enough to enable sufficient heat to penetrate therethrough to carry out the soldering operation, but is of sufficient thickness to prevent sufficient heat from passing into the metal of the rail to change its structure. Various 35 types of metal may be used in the plate 6 which is preferably formed of rolled material. For example, low carbon steel, austenitic stainless steel and copper have been used. In each case, plate 6 after its attachment to the rail will have a structure composed of small grains characteristic of worked metal in the portion adjacent the rail and a structure composed of large grains characteristic of the annealed metal in the remaining portion. The grains of the last portion will increase in size toward the surface thereof remote from the rail surface. If a steel 40 buffer plate is used the portion adjacent the rail has a structure composed of pearlite in a matrix of ferrite and the remaining portion a structure composed of martensite in a matrix of ferrite with the martensite content increasing in percentage toward the surface remote from the rail. In the case of copper, the portion of the plate adjacent the rail has a structure composed of elongated grains characteristic of worked copper and the portion 45 50 55 60 65 70

remote from the rail a structure composed of large equiaxed grains characteristic of annealed copper with the grains decreasing in size and changing from large equiaxed shape to elongated shape from the portion of the plate remote from the rail to the portion adjacent the rail. The thickness of plate 6 may vary somewhat but is preferably between about .035 and .050 inch.

While several embodiments of my invention have been shown and described it will be apparent that other adaptations and modifications may be made without departing from the scope of the following claims.

I claim:

1. The method of making and attaching a rail bond to a rail comprising placing a thin metal buffer plate against the rail with a soldering material between the plate and rail, placing a mold against the plate and around an electrical conductor, flowing molten metal into said mold to form a terminal fitting integral with the buffer plate and the conductor, said soldering material having a melting point lower than the melting points of said buffer plate and said molten metal, and correlating the heat of the molten metal, the heat penetration through the buffer plate and the melting temperature of the soldering material to cause the heat from the molten metal to solder the plate to the rail without changing the metallurgical structure of the rail.

2. A rail bond connection comprising an electrical conductor, a buffer plate having solder on the face thereof adjacent the rail, and a cast metal terminal integrally united with one end of said conductor and said buffer plate, said solder having a melting point lower than the melting points of said buffer plate and said cast metal, said buffer plate being interposed between

said conductor and said rail and having at least coextensive contact with said cast metal terminal, said cast metal terminal at least partially surrounding said conductor end, said buffer plate being connected to the said rail by said solder.

3. A rail bond connection according to claim 2 in which said buffer plate is made of steel with the portion thereof adjacent the rail having a structure composed of pearlite in a matrix of ferrite and the remaining portion a structure composed of martensite in a matrix of ferrite.

4. A rail bond connection according to claim 2 in which said buffer plate is made of copper with the portion thereof adjacent the rail having a structure composed of elongated grains characteristic of worked copper and the portion remote from the rail having a structure composed of large equiaxed grains characteristic of annealed copper.

References Cited in the file of this patent

UNITED STATES PATENTS

|           |              |       |               |
|-----------|--------------|-------|---------------|
| 656,125   | Kleinschmidt | ----- | Aug. 14, 1900 |
| 692,395   | Whiton       | ----- | Feb. 4, 1902  |
| 890,367   | Mead         | ----- | June 9, 1908  |
| 987,136   | Herrick      | ----- | Mar. 21, 1911 |
| 1,336,932 | Starkey      | ----- | Apr. 13, 1920 |
| 1,341,337 | Mead         | ----- | May 25, 1920  |
| 2,022,544 | Huber        | ----- | Nov. 26, 1935 |
| 2,225,028 | Banks        | ----- | Dec. 17, 1940 |
| 2,251,820 | Cadwell      | ----- | Aug. 5, 1941  |
| 2,318,604 | Febrey       | ----- | May 11, 1943  |
| 2,630,974 | Hicks        | ----- | Mar. 10, 1953 |